

## UNITED STATES PATENT OFFICE

2,305,745

## PROCESS OF PRODUCING LIGHT-SENSITIVE SYSTEMS

Ostap Stasiw, Dresden, Germany; vested in the Alien Property Custodian

No Drawing. Application June 3, 1940, Serial No. 338,641. In Germany June 15, 1939

6 Claims. (Cl. 95—7)

The invention relates to a process of producing light-sensitive systems, and particularly is directed to improvements in the light-sensitive substances, which are produced according to the process of my prior U. S. application, Ser. No. 306,896, filed Nov. 30, 1939.

The light-sensitive substances described in this prior application are produced by the introduction of alien sensitizing substances into metal halides, for example of silver sulfide into silver halide, and heating the mixture to a temperature at which said alien substance is incorporated into said silver halide by fusion, and in which the halogen liberated by dissociation during the heating is removed.

I have found, that the light-sensitive systems, produced according to the process of the above named prior application, are obtained in a particularly stable form by subjecting them to an additional oxidizing treatment which latter forms the principal object of the present invention. Moreover I have found, that it is possible, to vary and to regulate the light sensitiveness of these systems by this oxidizing treatment in a desired manner. Furthermore photographic emulsions, produced of colloids and of the oxidatively treated light-sensitive substances of the present invention, are very stable and do not fog, when developed.

Thus, the object of the invention is the oxidative treatment of the light-sensitive systems, produced according to the process of my U. S. application, Ser. No. 306,896, filed Nov. 30, 1939.

The oxidizing treatment of the light-sensitive substances may be carried out in a different manner. So the oxidizing treatment may be done during the production of the light-sensitive systems, or after it, employing high temperatures and high pressures if required. Oxidizing gases, such as oxygen, may be led over or through the molten mixture, stirring the same. Further the light-sensitive systems may be atomized by oxidizing gases or vapours, e. g. oxygen. By this treatment the light-sensitive systems are obtained as powders in a state of a very high fineness, especially useful for their technical application.

The invention is not limited to the oxidative treatment of the molten light-sensitive systems. Also the solid, light-sensitive systems may be treated in the same way, whereby the same good results are obtained.

Finally, the oxidizing treatment may be effected by working in an atmosphere of oxidizing

agents during the entire production process or in parts of it.

Oxidizing agents, that may be used in the process of the invention, are oxidizing gases or vapours, liquids, or solid substances, eventually such, which are able to give off oxidizing agents.

The temperatures used in the process and the duration of the oxidative treatment are dependent upon the nature and the desired properties of the light-sensitive systems and the nature of the oxidizing agent employed, and must be regulated in each case accordingly.

The light-sensitive products, prepared by the process of the invention, may be employed without binding substances. In such a case they are preferably cemented to suitable supports.

Further they may be introduced into colloids, serving as binding agents or carriers. Hereby emulsions are prepared, which are similar to the photographic emulsions. These mixtures of the light-sensitive products and the colloids may be poured as sheets, foils or the like, or may be applied on suitable supports.

The introduction of the light-sensitive systems into the colloids is done by carefully mixing them, e. g. by strongly stirring them, by treating them by vibrations, and/or by using the distributing, dispersing and wetting agents and processes which are known in colloidal chemistry.

The pouring of the emulsions of the light-sensitive substances and colloids in sheets or on supports may be effected by the usual methods of making photographic plates, films, papers and the like. The emulsions may be applied on one side of the support or both. They may be poured in one layer or more. Here, the usual measures in the manufacture of photographic plates, films, papers and the like are to be provided for, such as back-, adhering-, anti-halo-, filtering-, intermediary-, protecting- and covering layers. Also, optical photographic sensitizers and dyestuffs for coloring the layers may be added to the emulsions or incorporated in the layers, e. g. by bathing them in the solutions of the dyestuffs.

Colloids that may be used for the manufacture of the emulsions of the light-sensitive systems, are the different species of gelatine, among them also the so called "inert" gelatine, albumines and other proteins, collodion, cellulosic esters and ethers, natural and artificial resins and polymerisates, and the like.

As supports for the emulsions of the light-sensitive systems and the colloids, there may be used plates of glass, films of cellulose, collodion, cellulosic derivates, e. g. cellulosic esters or cel-

lulosic ethers, of resins or polymerisates, sheets of metals, paper and the like.

The powdering of the light-sensitive emulsions may be effected according to the methods known in the photographic industry for the production of photographic films, plates, and papers.

What I claim is:

1. In a method of producing light sensitive systems of silver halides, in which a mixture of silver halide and an alien substance acting as sensitizer is heated to a temperature at which said alien substance is incorporated into said silver halide by fusion and in which the halogen liberated by dissociation during the heating is removed, the additional step of subjecting the fused mixture which subsequently forms the light sensitive systems to an oxidizing treatment while still in its fused condition by treating the fused mixture with oxygen or oxygen containing gases.

2. In a method of producing light sensitive systems of silver halides, the steps of heating a mixture of silver halide and an alien substance acting as sensitizer to a temperature at which said alien substance is incorporated into said silver halide by fusion and in which the halogen liberated by dissociation during the heating is removed, subjecting the mixture, while in a molten condition, to an oxidizing treatment, and cooling the resulting product.

3. In a method of producing light sensitive systems of silver halides, in which a mixture of silver halide and an alien substance acting as sensitizer is heated to a temperature at which said alien substance is incorporated into said silver halide by fusion and in which the halogen liberated by dissociation during the heating is removed, the additional steps of treating the mixture, while still in a molten condition, with

oxygen which is led over the molten mixture, and cooling the resulting product.

4. In a method of producing light sensitive systems of silver halides, in which a mixture of silver halide and an alien substance acting as sensitizer is heated to a temperature at which said alien substance is incorporated into said silver halide by fusion and in which the halogen liberated by dissociation during the heating is removed, the additional steps of subjecting the mixture while still in a molten condition to an oxidizing treatment, by passing oxygen through the molten mixture, cooling the latter, and then comminuting the resulting solid product.

5. In a method of producing light sensitive layers of silver halides, including the steps of heating a mixture of silver halide and an alien substance acting as sensitizer to a temperature at which said alien substance is incorporated into said silver halide by fusion and in which the halogen liberated by dissociation during the heating is removed, then atomizing the fused mixture by an oxidizing gas and incorporating the finely disintegrated light sensitive systems thus produced into a colloidal carrier.

6. In a method of producing light sensitive layers of silver halides, in which a mixture of silver halide and an alien substance acting as sensitizer is heated to a temperature at which said alien substance is incorporated into said silver halide by fusion and in which the halogen liberated by dissociation during the heating is removed, the additional steps of subjecting the mixture while still in a molten condition to an oxidizing treatment, cooling the oxidized mixture, and incorporating the light sensitive systems thus produced in a finely disintegrated condition into a colloidal carrier.

OSTAP STASIW.